

# United States Patent Office

3,284,206

Patented Nov. 8, 1966

1

3,284,206

## IMAGE YIELDING LAYERS

Ralph Kingsley Blake, Westfield, N.J., assignor to E. I. du Pont de Nemours and Company, Wilmington, Del., a corporation of Delaware  
No Drawing. Filed Oct. 13, 1964, Ser. No. 403,661  
10 Claims. (Cl. 96—107)

This application is a continuation-in-part of Blake Ser. No. 236,420, applicant's prior application filed Nov. 8, 1962, and issued Nov. 3, 1964, as U.S. Patent 3,155,507.

This invention relates to photography and more particularly to new image-yielding photographic silver halide emulsion layers and to photographic elements embodying such layers.

The principal processes of photography are based on the use of colloid-silver halide emulsion layers. In the prior art processes a latent image is formed by image-wise exposure of a radiation-sensitive silver halide emulsion layer. Silver halide bearing a latent image has been developed to silver by selective reduction in these instances. In the prior processes of photography the unreduced silver remaining after development has been removed by silver halide solvents or rendered insensitive or transparent by treatment with complexing agents. Optional after-treatments include intensification, reduction, toning and tinting. However, the primary or first step in image formation always has been based on the selective reduction step.

An entirely different type of photographic process has been described in assignee's copending application of Blake, U.S. Ser. No. 236,420, filed Nov. 8, 1962. The novel process of said application, characterized as "photosolubilization," requires the use of a specially prepared silver halide emulsion layer containing a stipulated amount of an organic compound which modifies the silver halide solubility so that, in conventional silver halide solvents, said organic compound causes the silver halide grains to dissolve more slowly than normal. Such an element is given an image-wise exposure and the exposed areas can then be treated in a solution of a silver halide solvent to yield a positive, silver halide image (the silver halide remaining undissolved in the unexposed areas). As an optional additional processing step, the silver halide image may be intensified, e.g., by reduction, to convert it into a black, metallic silver image.

It is an object of this invention to provide new photographic silver halide compositions, photographic layers, and photographic elements bearing a layer of silver halide. Another object is to provide processes for making these products. A further object is to provide such products which are adapted to more versatile processes for forming silver and other images and which are simple, dependable and give results equal in quality to the prior conventional methods. A more particular object is to provide new compositions and elements for "photosolubilization" processing embodying a class of organic compounds which provide a new combination for the required alteration of the silver halide crystals. Still further objects will be apparent from the following description of the invention.

The above objects are realized in a photographic emulsion layer comprising, before exposure to actinic radiation, light-sensitive silver halide crystals having associated therewith a silver selenide of a selenyl compound (selenol) of the formula:



where  $R_1$  is an organic radical, said silver selenide being of lower solubility in water than silver chloride and the silver halide crystals so associated with the silver selenide dissolving more slowly in a 10% by weight aqueous sodium thiosulfate solution at a predetermined pH, than untreated silver halide crystals.

2

It is preferred that the selenide be present in such an amount, in terms of the ratio of its weight to the surface area of said silver halide crystals, that when admixed in such ratio with an aqueous silver chlorobromide (70/30 mole percent) gelatin dispersion containing 10 g. of gelatin per mole of Ag and .57 mg. of Ag per ml., and said silver chlorobromide dispersion is treated with 10%, by weight, aqueous sodium thiosulfate (so that the resulting mixture contains 0.29 mg. of silver and 100 mg. of sodium thiosulfate), at least three times the amount of silver chlorobromide remains undissolved as in a similar dispersion successively treated with 5%, by weight, aqueous sodium hypochlorite and 10%, by weight, aqueous sodium thiosulfate (so that the resulting mixture contains 0.29 mg. of silver, 25 mg. of sodium hypochlorite and 100 mg. of sodium thiosulfate), after vigorous agitation of both dispersions for 30 seconds at 25°C.

In an important embodiment of the invention, the organic selenyl compound has the formula:



where  $R$  and  $R'$ , which may be the same or different, are 25 hydrogen, hydrocarbon or substituted hydrocarbon nuclei of 1-14 carbons, i.e., alkyl, aryl, alkaryl, aralkyl radicals, and such radicals containing substituent groups such as nitro, halogen, e.g., chlorine and bromine, alkoxy of 1-6 carbon atoms. When separate, at least one radical  $R$  or 30  $R'$  is hydrocarbon of 3-14 carbons. When  $R$  and  $R'$  are taken together, they form an aromatic or alicyclic ring. The silver salt of the selenol is of less solubility in water than silver chloride and the silver halide crystals so associated with the said silver salt dissolve more slowly in 35 10% aqueous sodium thiosulfate solution, at a predetermined pH, than untreated silver halide crystals.

$R'$  of Formula 2 preferably is H, and  $R$  is an unsubstituted hydrocarbon radical of 6-10 carbon atoms and has a cyclic hydrocarbon radical of 6 carbon atoms attached through a cyclic carbon of said radical to the 4-carbon atom of the thiazole ring. Suitable radicals of the latter type include cyclohexyl, phenyl, and alpha-naphthyl.

Preferably, the silver halide crystals are dispersed in 45 a water-permeable organic colloid to form a light sensitive photographic emulsion. The selected selenyl compound can be added to the silver halide emulsion while the latter is in the liquid state or the emulsion may be 50 coated on a suitable support and the resulting element bathed or impregnated with a solution, e.g., an alcoholic solution of the organic compound. The desired amount of the selenyl compound in the silver halide emulsion may vary with a number of factors such as the nature 55 of the selenyl compound and the size of the silver halide crystal (and thus the surface area of the crystal per mole of silver halide).

When the selenol is added to the emulsion in the liquid state it is most efficiently adsorbed to the silver halide crystals by "digesting" the emulsion, i.e., heating the emulsion between 140 and 180°F. The selenol is used in greater than fog-inhibiting amounts, e.g., from 0.3 to 1.5 grams per mole of silver halide and, more preferably, from 0.4 to 1.2 grams per mole of silver halide. The optimum concentration of selenol is decreased somewhat, e.g., about 10%, when the emulsion is sensitized with a photographic optical sensitizing dye as disclosed in assignee's copending application of Blake, Ser. No. 390, 460, filed August 18, 1964.

The gelatin-silver halide ratio is quite flexible and may 70 vary from 3:1 to 1:20 depending on the particular organic compound and application.

In an important use of the products of the invention, direct positive images are formed by a process which comprises:

(a) Exposing imagewise to actinic radiation a photo-sensitive layer comprising silver halide crystals treated with the selenol as described above.

(b) Treating the exposed layer in a solution of a silver halide solvent to remove soluble silver halide in the exposed image areas, thus forming a positive silver halide image, and optionally,

(c) Washing the resulting layers. If desired, the silver halide image may be viewed directly, e.g., by projection (if on a transparent support) or it may be intensified, e.g., by

(d) Converting the residual silver halide to silver by treatment in a fogging developer, e.g., a high pH, 1-phenyl-4-methyl-3-pyrazolidone/hydroquinone developer containing iodide ion or by fogging the emulsion by exposure to light and then treating with a silver halide reducing agent, e.g., a conventional silver halide developer, and

(e) Washing the developed layer to reveal a positive silver image in the original non-exposed areas.

The imagewise solution of the exposed silver halide/selenol stratum may be effected by the silver halide solvents commonly used as photographic fixing agents, e.g., sodium thiosulfate, sodium thiocyanate concentrated solutions of potassium bromide, etc. In assignee's copending application Hunt, Ser. No. 388,919 filed August 11, 1964, it is disclosed that more efficient removal of exposed silver halide crystals (insolubilized by mercapto compounds) may be obtained when the fixing solution contains an inorganic cation selected from the class consisting of potassium, cesium, rubidium, thallium (I) strontium, and lead (II). These cations are also effective as additives for fixing solutions used in treating the elements of this invention.

Reduction of the treated residual silver halide may be accomplished by the use of any chemical reducing agent capable of reducing silver ion to silver metal, e.g., hydroquinone, metol, sodium hydrosulfite and stannous chloride. The function of the reducing agent may be enhanced by modifying the surface properties of the treated, residual silver halide crystals by means of alcohol, thiourea, potassium iodide, etc. The silver halide image may be toned, e.g., with sodium sulfide, sodium selenide, etc. In addition, color images may be obtained by developing the treated, residual silver halide with a primary aromatic amine color developing agent in the presence of a color coupling compound either in the developing bath or previously incorporated in the emulsion. Additionally, the silver halide image may be intensified by dye mordanting.

The present invention is not limited to a narrow class of selenols with which the silver halide crystals are intimately associated or may be treated in preparing the novel compositions of this invention. Instead, a large number of useful compounds can be employed and their utility can be readily determined by a relatively simple test. Essentially, the test consists of two steps. Test A and Test B. In Test A, the candidate selenol must render a dispersion of silver halide crystals insoluble in a silver halide solvent, i.e., an aqueous solution of sodium thiosulfate, at some pH between 1 and 13. If the candidate compound meets the insolubility requirements of Test A, it must also meet the requirements of Test B by forming with said dispersion of silver halide crystals a reaction product which, upon treatment with an aqueous solution of sodium hypochlorite, becomes soluble when subsequently treated with aqueous sodium thiosulfate. The following practical tests are provided in further exemplification of the invention and include specific concentrations of solutions, times, etc., so that suitable selenols may be readily and positively identified.

#### TEST A

A solution, nearly saturated at 25° C. with a candidate selenol, is prepared using ethanol, acetone, dimethyl

formamide, water or other suitable solvent. Depending on the solubility, a solution concentration from 0.01 to 10 percent by weight is obtained. Twenty-five ml. of a silver chlorobromide dispersion containing 25 mg. of silver halide (calculated as silver bromide), prepared as described below, is treated with small increments (i.e., about 0.1 to 0.2 ml. at a time) of the said candidate solution under safelight conditions (Wratten 1A filter or equivalent) until the silver halide dispersion either is rendered insoluble in 10% aqueous sodium thiosulfate or the candidate is found not to cause insolubilization. Generally insolubilization will occur upon the addition of 0.05 g. or less of said candidate selenol, calculated as the pure compound. Compounds which must be used in substantially greater quantities than this, e.g., 1-2 g., to effect insolubilization are considered less preferred compounds. The silver halide dispersion insolubility is determined by taking a 0.5 ml. portion of the silver halide dispersion (after each incremental addition of the candidate selenol), adding about 0.1 to 0.2 ml. of 10% aqueous sodium thiosulfate solution and observing the turbidity after 30 seconds.

As a control, one should use 25 ml. of water to which small increments of the candidate solution are added. Half-milliliter portions of the control are treated in the same manner with the sodium thiosulfate solution. The presence of visual turbidity relative to the control is sufficient to satisfy the definition of insolubility in this test.

This test may be repeated for various pH increments from 1 to 13. Although there is some optimum pH value at which the test is most sensitive, this is not a sharp maximum which must be precisely attained. Rather, it has been found that there is a fairly broad range of pH values (e.g., 2.0 to 3.0 pH units) over which the test has a satisfactory sensitivity. In practice, the silver halide dispersion might be tested without adjustment (e.g., at pH 5.0 to 7.0) and if insolubilization occurs here, Test A is completed. If there is no insolubilization, the test is repeated at a higher pH (e.g., from pH 10-13). If there is still no insolubilization, the test is conducted with the emulsion adjusted to a lower pH (e.g., about pH 1-3). Thus three different pH values represent a practical maximum number which must be investigated to determine whether or not insolubilization will occur.

#### TEST B

A selenol capable of insolubilizing a silver halide dispersion according to Test A is now ready for the next test, which again will be conducted under safelight conditions. To the above silver halide dispersion, there is added the minimum amount of a solution of the candidate selenol found necessary for insolubilization. Half-milliliter samples of the dispersion containing 0.5 mg. of AgBr or 0.29 mg. of Ag are placed in two test tubes. To one sample is added 0.5 ml. of water; to the other is added 0.5 ml. of a 5% by weight aqueous solution of sodium hypochlorite (25 mg. NaOCl). Next, there is added to both samples, 1.0 ml. of an aqueous 10% by weight solution of sodium thiosulfate (100 mg. thiosulfate). If, after standing for up to thirty seconds, the sample treated with sodium hypochlorite clarifies (or becomes less turbid) relative to the control sample, the candidate selenol meets the requirements of Test B and is satisfactory for use in accordance with this invention. The chemical testing for selecting suitable compounds has been found to give absolute correlation, i.e., organic compounds which have been subjected to Tests A and B have produced without exception, when tested in actual photographic emulsions, the very effects predicted by said tests.

The silver chlorobromide dispersion referred to in the above test is a lithographic emulsion having a silver halide composition of 30 mole percent AgBr and 70 mole percent AgCl and having 20 grams of gelatin present per mole of silver halide for the steps of precipitation and ripening. This emulsion was freed of unwanted, soluble,

by-product salt by a coagulation and wash procedure as taught in Waller et al., U.S. Patent 2,489,341, wherein the silver halide and most of the gelatin were coagulated by an anionic wetting agent, sodium lauryl sulfate, using an acid coagulation environment. Following the washing step, the emulsion coagulant was redispersed in water. Assuming a loss of 10 grams of gelatin per mole of silver halide during washing, the final gelatin concentration was about 10 grams per mole of silver halide. For use in the above test, the dispersion was diluted to the extent that one milliliter of dispersion contained one mg. of silver halide (calculated as AgBr, or 0.58 mg. of Ag).

Dispersed crystals of silver halide, treated with an appropriate amount of a suitable selenol, are affected by exposure of a portion of said crystals to actinic radiation, e.g., ultraviolet, visible, infrared, X-radiation, etc., to such an extent that at least 20% of the less soluble (unexposed) crystals remain when 90% of the more soluble (exposed) crystals dissolve when treated in 10% by weight aqueous sodium thiosulfate solution.

Suitable elements in this invention can be prepared by bathing a photographic film in a solution of an appropriate selenol. In this embodiment, the silver halide crystals near the surface of the coated emulsion stratum are in contact with a higher concentration of the selenol. Crystals farther from the surface are treated with less of the selenol and, if the rate of diffusion is sufficiently slow, there may be considerably less of the selenol (even approaching zero) reacting with the lower than with the surface silver halide crystals. In such elements, satisfactory results might be obtained with only a fraction, e.g., one-half of the amount of the selenol theoretically calculated as required to just cover the surface of a mole of the silver halide crystals.

The invention will be further illustrated by, but is not intended to be limited to, the following examples.

#### Example I

##### 2-SELENYLBENZOTHIAZOLE

To a solution of sodium selenide (25 g., 0.2 moles) in 250 ml. of water, under a nitrogen atmosphere, are added 33.9 g. (0.2 mole) of 2-chlorobenzothiazole and with rapid stirring the mixture is then heated to reflux. The mixture is maintained at gentle ebullition for a period of 30 to 45 minutes until droplets of the 2-chlorobenzothiazole disappear in the reflux. The 2-selenylbenzothiazole (yellow crystals of melting point 140-143° C.) is then precipitated from the solution of its sodium salt with an acidifying agent, sulfuric acid.

A lithographic emulsion containing about 10 g. of gelatin per mole of silver halide (prepared as described following Test B) plus 47 g. of gelatin, was adjusted to 2320 g. by addition of water and the temperature was adjusted to 110° F. The 2-selenylbenzothiazole, prepared as described above, was added to the emulsion from a 1% by weight ethanol solution in the amount of 1.26 g. per mole of silver halide. The emulsion was digested for 20 min. at 160° F. and then cooled to 95° F. Chrome alum hardener and other emulsion adjuvants were added as final additions. This emulsion was applied at a coating weight of 70 mg. of silver halide (calculated as AgBr) per square decimeter on 0.004-inch thick polyester photographic film base as described in Example IV of Alles U.S. 2,779,684. The coating, after imagewise exposure, showed a greater rate of dissolution in a 1.0 N (0.5 molar) aqueous sodium thiosulfate solution in the exposed areas than in the unexposed areas so as to form a positive silver halide image. Subsequent flashing to white light, followed by treatment with a reducing agent (a conventional photographic developing solution containing 1-phenyl-4-methyl-3-pyrazolidone and hydroquinone), resulted in the formation of an intensified positive image of metallic silver.

#### Example II

##### SELENOPHENOL

Commercially available selenophenol was tested according to the above-described Test A and it produced the required insolubilization of silver halide crystals. Chemical solubilization also occurred according to Test B as described above. More quantitative results were obtained by applying Test C, a simulated photographic test as described below:

##### TEST C

A 0.5 ml. portion of the insolubilized dispersion prepared in Test A under safelight conditions is placed in a 12x75 mm. heat-resistant glass tube 3 inches from a high-intensity tungsten filament incandescent lamp (General Electric Reflector Photoflood Lamp, No. PH/RFL2). This insolubilized dispersion is exposed to the lamp for up to 10 minutes. A control consisting of another 0.5 ml. portion of the insolubilized silver halide dispersion from Test A is taken under safelight conditions. Two-tenths of a milliliter of 10% aqueous sodium thiosulfate is added to each of the dispersion samples which are compared under safelight conditions. Any reduction in turbidity of the dispersion exposed to the photoflood lamp compared to the unexposed control after treatment with aqueous sodium thiosulfate solution shows that photosolubilization occurs.

In this more quantitative Test C, it was determined that the approximate minimum quantity of selenophenol required to insolubilize 25 milligrams of silver halide was 0.4 milligram.

#### Example III

##### 2-SELENYLBENZOSELENAZOLE

According to a procedure like that described in the Example I, 2-selenylbenzoselenazole was prepared using 2-chlorobenzoselenazole in place of the 2-chlorobenzothiazole of that example.

A photographic element was prepared by coating an aqueous gelatin dispersion of silver chlorobromide (70 mole percent silver chloride and 30 mole percent silver bromide) on a film base prepared as described in Example IV of Alles U.S. Patent 2,779,684. The dispersion had a ratio of silver halide to gelatin of 19:1 by weight and was coated at a pH of 6 at a rate of 116 milligrams of silver halide per square decimeter. After drying, the element was bathed for about 30 seconds in an ethanol-water solution of 2-selenylbenzoselenazole and dried. The solution of 2-selenylbenzoselenazole was prepared by diluting 5 ml. of a stock solution (1 gram of the compound made up to 100 ml. in ethanol) with an additional 20 ml. of ethanol and 10 ml. of water. The dried element was then exposed behind a photographic transparency for 5 seconds to the radiation from the lamp described in Example II spaced at a distance of about 6 inches. The exposed element was then immersed in a solution containing, on a liter basis, 77 g. Na<sub>2</sub>S<sub>2</sub>O<sub>3</sub>, 7.5 g. Na<sub>2</sub>SO<sub>3</sub>, 9 g. Na<sub>2</sub>B<sub>4</sub>O<sub>7</sub>·10H<sub>2</sub>O, 6 ml. glacial acetic acid, 10 g. KAl(SO<sub>4</sub>)<sub>2</sub>·12H<sub>2</sub>O and 10 g. CH<sub>3</sub>COOK. A 30-second treatment in this solution resulted in the removal of the silver salt in the exposed areas. Subsequently, the fixed film was then rinsed briefly in water and bathed in a rapid acting fogging photographic developer solution comprising 1-phenyl-4-methyl-3-pyrazolidone and hydroquinone as reducing agents to which there had been added potassium iodide and a direct positive image formed. All of the above operations were carried out under red safelight illumination.

#### Example IV

##### 2-SELENYLBENZOXAZOLE

The above compound was prepared according to the procedure of Example I except for using 2-chlorobenzoxazole in place of the 2-chlorobenzothiazole of that example. 2-chlorobenzoxazole is commercially available. The

selenyl compound thus prepared was tested as a treating solution for a photographic element as described in Example III and a similar positive image was obtained.

This selenol also caused the required insolubilization of silver halide crystals according to Test A and the required chemical solubilization according to Test B. In Test C it was determined that the approximate minimum quantity of 2-selenylbenzoxazole required to insolubilize the 25 mg. of silver halide was 1.0 mg.

*Example V*

**2-SELENYL-4-PHENYLTHIAZOLE**

2-bromo-4-phenylthiazole was prepared according to the procedure of Ralhan et al., J. Indian Chem. Soc., vol. 37, No. 12 (1960) page 773-4. One-tenth of a mole of this compound was added to a slight excess of an ether solution of n-butyllithium at -10° to -20° C. (using a Dry Ice-acetone bath). After about an hour and a half of stirring at this temperature, the reaction mixture was cooled to -40° C. and 0.1 mole of powdered selenium was added. The reaction mixture was then stirred while allowing it to warm to about 0° C., then the mixture was poured onto ice. Upon acidification with H<sub>2</sub>SO<sub>4</sub> the desired compound, 2-selenyl-4-phenylthiazole was isolated from the separated ether layer.

The resulting compound, was tested as a treating solution for a photographic element as described in Example III and a similar positive image was obtained.

This selenol also caused the required insolubilization of silver halide crystals of Test A and the required chemical solubilization of Test B. In Test C it was determined that the approximate minimum quantity of 2-selenyl-4-phenylthiazole required to insolubilize the 25 mg. of silver halide was 0.3 mg.

*Example VI*

**2-SELENYL-4-CYCLOHEXYLTHIAZOLE**

The above compound was prepared using a procedure very similar to that of Example V except for the substitution of 2-bromo-4-cyclohexylthiazole in place of 2-bromo-4-phenylthiazole.

The resulting compound was tested as a treating solution for a photographic element as described in Example III and a similar positive image was obtained.

*Example VII*

**2-SELENYL-4-AMYLTHIAZOLE**

The above compound was prepared using a procedure very similar to that of Example V except for the substitution of 2-bromo-4-amylthiazole in place of 2-bromo-4-phenylthiazole.

The resulting compound was tested as a treating solution for a photographic element as described in Example III and a similar positive image was obtained.

*Example VIII*

**1-SELENYLOCTANE**

1-selenyloctane was prepared from normal bromooctane by reaction with sodium selenide under nitrogen. The resulting compound was tested as a treating solution for a photographic element as described in Example III and a similar positive image was obtained.

A number of other selenols of the structure R—SeH can be synthesized according to procedures similar to those described above and can be used in the preparation of photosolubilizable compositions and elements to give photographic results as described in the above examples. Such compounds include:

- 2-selenyl-4-(p-bromophenyl) thiazole
- 2-selenyl-4-(p-methoxyphenyl) thiazole
- 2-selenyl-4-(p-ethylphenyl) thiazole
- 2-selenyl-4-(p-chlorophenyl) thiazole

The silver halide need not be a combination of silver chloride and silver bromide, but may be silver chloride, silver bromide and other mixed halide systems conventional in photographic practice, e.g., silver bromoiodide. 5 While, for rapid processing, a high silver halide to binder ratio is desirable, more conventional ratios can also be used.

In place of part of the gelatin, other natural or synthetic water-permeable organic colloid binding agents can be used and in some cases such binders can be used alone. 10 Such agents include water-permeable or water-soluble polyvinyl alcohol and its derivatives, e.g., partially hydrolyzed polyvinyl acetates, polyvinyl ethers and acetals containing a large number of intralinear



groups, hydrolyzed interpolymers of vinyl acetate and unsaturated addition polymerizable compounds such as maleic anhydride, acrylic and methacrylic acid esters and styrene. 20 Suitable such colloids of the last-mentioned type were disclosed in U.S. Patents 2,276,322; 2,276,323 and 2,397,866. The useful polyvinyl acetals include polyvinyl acetaldehyde acetal, polyvinyl butyraldehyde acetal and polyvinyl sodium o-sulfobenzaldehyde acetal. Other 25 useful colloid binding agents which can be used include the poly-N-vinylactams of Bolton U.S. Patent 2,495,918, various polysaccharides, e.g., dextran, dextrin, etc., the hydrophilic copolymers in Shacklett U.S. Patent 2,833,650, hydrophilic cellulose ethers and esters, and polymers of 30 acrylic and methacrylic esters and amides. Also, it has been found practical to treat silver halide layers on a base material in the essential absence of a binder, e.g., those prepared by chemical or vacuum deposition.

The emulsion may optionally contain any of the 35 usual adjuvants customarily employed in silver halide systems so long as they do not interfere with the absorption and complexing action of the selenomercaptans of the invention.

The emulsions can be coated on any suitable support, 40 e.g., cellulose esters, cellulose mixed esters; superpolymers, e.g., poly(vinyl chloride co vinyl acetate); polyvinyl acetals, butyral; polystyrene; polyamides, e.g., polyhexamethylene adipamide, polyesters, e.g., polycarbonates, polyethylene terephthalate/isophthalate, esters 45 formed by condensing terephthalic acid and its derivatives, e.g., dimethyl terephthalate with propylene glycol, diethylene glycol, tetramethylene glycol, cyclohexane-1,4-dimethanol (hexahydro-p-xylene dialcohol); paper, metal, glass, etc.

The novel photographic compositions of this invention 50 have numerous advantages. One advantage is the simplicity of their preparation. The photographic processes applicable to the compositions of the invention likewise have advantages over previously known systems based on selective reduction of exposed silver halide for forming either direct positive or negative images without resorting to the special effects and sensitizing procedures previously used for preparing such images. In addition, 55 since direct positive image formation does not require selective reduction, this process is not limited to the use of certain photographic developing agents but may be accomplished by using a wide range of reducing agents. Many such compounds are of very low cost and can be used to form images of much higher covering power than 60 customary, thus effecting important economies in processing, as well as greatly increasing the efficiency of the silver image.

Another advantage of this invention is that it provides 65 new elements for forming silver images that do not require special equipment and apparatus. A further advantage is that the elements can be used successfully by photographic technicians and photographers of ordinary skill. A still further advantage is that the elements can be processed with conventional reducing agents, e.g., developers 70

and fixing agents. Still additional advantages will be apparent from the above description of the invention.

What is claimed is:

1. A photographic emulsion layer comprising, before exposure to actinic radiation, light-sensitive silver halide crystals having associated therewith in greater than fog-inhibiting amounts a silver selenide of a selenyl compound of the formula



wherein  $R_1$  is an organic radical that is attached to the Se atom by a carbon atom; said silver selenide being of lower solubility in water than silver chloride, the silver halide crystals so associated with the silver selenide dissolving more slowly in 10% aqueous sodium thiosulfate than untreated silver halide crystals at a predetermined pH, the selenyl compound of said formula being present in such amount, in terms of the ratio of its weight to the surface area of said silver halide crystals, that when admixed in such ratio with an aqueous silver chlorobromide (70/30 mole percent) gelatin dispersion containing 10 g. of gelatin per mole of Ag and .57 mg. of Ag per ml., and said silver chlorobromide dispersion is treated with 10%, by weight, aqueous sodium thiosulfate (so that the resulting mixture contains 0.29 mg. of silver and 100 mg. of sodium thiosulfate), at least three times the amount of silver chlorobromide remains undissolved as compared with a similar dispersion successively treated with 5%, by weight, aqueous sodium hypochlorite and 10%, by weight, aqueous sodium thiosulfate (so that the resulting mixture contains 0.29 mg. of silver, 25 mg. of sodium hypochlorite and 100 mg. of sodium thiosulfate), after vigorous agitation of both dispersions for 30 seconds at 25° C.

2. An emulsion layer according to claim 1 wherein gelatin is present as a binding agent for said crystals.

3. An emulsion layer according to claim 1 wherein the silver halide is silver chlorobromide.

4. An emulsion layer according to claim 1 wherein the silver halide is silver chloride.

5. A photographic emulsion layer comprising before exposure to actinic radiation light-sensitive silver halide crystals having associated therewith in greater than fog-inhibiting amounts a silver selenide of a selenyl compound of the formula



where  $\text{R}$  and  $\text{R}'$  are members selected from the group consisting of hydrogen and hydrocarbon nuclei of 1-14 carbon atoms connected through carbon to the thiazole

ring, at least one of  $\text{R}$  and  $\text{R}'$  when separate being a hydrocarbon nucleus of 3-14 carbon atoms and when taken together constituting the atoms necessary to complete with the two carbon atoms of the thiazole ring a cyclic radical; said silver selenide being of lower solubility in water than silver chloride, the silver halide crystals so associated with the silver selenide dissolving more slowly in 10% aqueous sodium thiosulfate than untreated silver halide crystals at a predetermined pH, the selenyl compound of said formula being present in such amount, in terms of the ratio of its weight to the surface area of said silver halide crystals, that when admixed in such ratio with an aqueous silver chlorobromide (70/30 mole percent) gelatin dispersion containing 10 g. of gelatin per mole of Ag and .57 mg. of Ag per ml., and said silver chlorobromide dispersion is treated with 10%, by weight, aqueous sodium thiosulfate (so that the resulting mixture contains 0.29 mg. of silver and 100 mg. of sodium thiosulfate), at least three times the amount of silver chlorobromide remains undissolved as compared with a similar dispersion successively treated with 5%, by weight, aqueous sodium hypochlorite and 10%, by weight, aqueous sodium thiosulfate (so that the resulting mixture contains 0.29 mg. of silver, 25 mg. of sodium hypochlorite and 100 mg. of sodium thiosulfate), after vigorous agitation of both dispersions for 30 seconds at 25° C.

6. An emulsion layer according to claim 5 wherein gelatin is present as a binding agent for said crystals.

7. An emulsion layer according to claim 5 wherein the silver halide is silver chlorobromide.

8. An emulsion layer according to claim 5 wherein the silver halide is silver chloride.

9. An emulsion layer according to claim 5 wherein the selenyl compound is 2-selenylbenzothiazole.

10. An emulsion according to claim 5 wherein the selenyl compound is 2-selenyl-4-phenylthiazole.

#### References Cited by the Examiner

#### UNITED STATES PATENTS

- 2,195,150 3/1940 Kendall ----- 96-109  
3,161,508 12/1964 Hepher et al. ----- 96-33 X

#### References Cited by the Applicant

#### UNITED STATES PATENTS

- 2,520,358 8/1950 Brooker.  
3,155,507 11/1964 Blake.

50 NORMAN G. TORCHIN, Primary Examiner.

J. TRAVIS BROWN, Examiner.

D. D. PRICE, Assistant Examiner.